

J. C. NICHOLLS.  
SMOKELESS POWDER.  
APPLICATION FILED FEB. 21, 1916.

1,208,358.

Patented Dec. 12, 1916.

Fig. 1.



Fig. 3.



Fig. 2.



Fig. 5.



Fig. 4.



Fig. 7.



Fig. 6.

Inventor

JESSE C. NICHOLLS

*Jesse C. Nicholls*

Attorneys.

# UNITED STATES PATENT OFFICE.

JESSE C. NICHOLLS, OF THE UNITED STATES ARMY.

## SMOKELESS POWDER.

1,208,358.

Specification of Letters Patent. Patented Dec. 12, 1916.

Application filed February 21, 1916. Serial No. 79,711.

To all whom it may concern:

Be it known that I, JESSE C. NICHOLLS, a citizen of the United States, residing at Picatinny Arsenal, Dover, county of Morris, State of New Jersey, have invented new and useful Improvements in Smokeless Powders, of which the following is a specification.

My invention relates to an improvement 10 in smokeless powders, with the object in view of obtaining a finished product which can be used in firing from cannon, blank charges or charges with very little tamping, without the usual projectile, and will, when 15 so fired, produce a loud report similar to that obtained when firing takes place with ammunition consisting of the usual propelling charge of powder and a projectile.

My invention is herewith fully described 20 and pointed out in the claims.

For convenience, the term "maneuver powder" will hereinafter be used to designate powders which, when fired without high resistance such as that imposed by the 25 usual projectile, are capable of producing a loud report attended by small amounts of smoke or visible vapors, and thus simulate the regular service round of smokeless powder and projectile as to report and appearance.

Heretofore, attempts have been made to use, for maneuver powders, the following powders, among others, in some instances separately, and in others mixed together, to 30 wit:—(a) Small arms rifle powders, both of the straight nitrocellulose type and of the nitrocellulose-nitroglycerin type, separately, or in combination with each other.

(b) Certain pistol powders, such as those 40 known, commercially, under the names "Bullseye" or "Pistol No. 1." (c) Quick burning powders, such as those known commercially as "Shotgun," "Bulk" and "New Schultze." (d) Nitrated blotting, 45 filter, and tissue papers partly colloided or partly dissolved, in various degrees, by the different known solvents for nitrocellulose or cellulose nitrate. (e) Powders made of cellulose nitrate of different nitrogen contents, either alone or mixed one with another, colloided or partly dissolved with different solvents, pressed into thin walled hollow cylinders and cut so that the grains 50 were about two or three times as long as their outside diameter. (f) So-called "Thorn Maneuver Powder" procured from

Europe, the method of manufacturing which is not definitely known to the public, but which appears to be nitrated paper partly colloided or dissolved and then dried. 60

(g) Single perforated cord of powder, in constituency like that used in the U. S. magazine rifle, Cal. .30, but differing in form, in that it was cut to a short length of only about one two-hundredths of an inch. 65

(h) Nitrocellulose powder extruded from the graining press in the form of long, very thin, flat ribbons. (i) The above powders combined with ordinary fine grained charcoal powders, with mealed charcoal powders, 70 or with partially smokeless powders such as Du Pont "Lesmok" and others of similar composition.

The powders or combinations of powders 75 enumerated above have without exception, been not very suitable, or entirely unsuitable for use as maneuver powders for one or more of the following reasons: Report not loud enough; too much smoke produced; high or irregular pressures; loss of chemical 80 stability with age; space occupied by the appropriate charge so small as to allow interference between a long primer and the closing wad that holds the powder in the case; small space occupied by the appropriate charge rendering liable the use of a 85 dangerously large charge, due to error in weighing, measuring or otherwise selecting the amount of the powder to be used in the charge. 90

The object of my invention, as set forth above, is attained by a particular method of cutting up or subdividing powder of suitable constituency, which will be understood 95 from the following: Rods, cords, or other convenient forms of powder of the same compositions or similar in general to any of the usual smokeless powders, are preferably the material employed and subjected to the novel method of subdivision. Some of these 100 are composed of: Cellulose nitrate or nitrocellulose, sometimes called gun cotton when high in nitration (13.20% of nitrogen), or pyrocellulose when comparatively low in nitrogen (12.60% of nitrogen), mixed or 105 colloided with mixture of ether and alcohol, nitroglycerin, nitroglycerin and acetone, amyl alcohol, amyl acetate, ethyl acetate or other such solvents or mixtures of solvents. However, I do not limit myself to cellulose 110 nitrates of the above percentages of nitrogen, as the percentages may vary greatly

from those given above, neither do I limit myself to the ingredients mentioned.

One convenient way to proceed is to mix the ingredients and run the mixture through the usual blocking presses and graining press, so as to convert it into a colloidal form generally similar to that ready to be cut into grains in making ordinary propelling smokeless powders. The extruded 10 rod or cord is then cut into such lengths that the pieces may be placed conveniently in appropriate machines, hereinafter described, for again cutting them to their final form, after which the resulting powder may 15 be dried if necessary so that it is ready for use in firing blank rounds.

This powder may be cut to its finished form immediately after being pressed into rods or cords, while it is "green"—that is, 20 still contains a great amount of the solvents or other volatiles. It also may be cut to finished form at any degree of dryness from the green state to the state usually known as completely dry, in which latter state the 25 solvents or other volatiles originally contained in the powder have evaporated away until only a small percentage of them remains in the pieces to be cut. As an illustration, the rods may be cut to finished product while they contain anywhere from 5% or less to about 50% of volatiles and solvent. I do not limit myself to these percentages, but can use percentages both higher and lower than those given. The rods, cords, or other 30 shapes are then, by the use of suitable tools or machines, cut or shaved into disks, sheets or ribbons, comparatively very thin, that is to say, with a thickness very small as compared to the dimensions in the plane of the 35 section such as diameter, or length and breadth of the shaving. I am aware that powders have been made by rolling, pressing or cutting so that the least dimension is much less than the other two dimensions. 40 However, in none of those powders have the ratios of least dimension to the other dimensions been small enough to make those powders suitable for use as maneuver powders. For instance, the pistol powders 45 known as "Bullseye" and "Pistol No. 1" consist of grains in the form of thin disks. When first cut these disks are only about one three hundred and fiftieth of an inch thick, and the diameter of the disks is about 50 five one-hundredths of an inch.

For maneuver powder made in accordance with this patent specification, the ratio of the thickness to the other two dimensions is much less than for the "Bullseye" or 60 "Pistol No. 1." In accordance with my invention herein described, the maneuver powder may be cut in the following way among others: Rods about two feet long, and with a diameter of from one-half inch 65 to two inches, with or without one or more

longitudinal perforations, are placed in a lathe, so as to rotate, while an ordinary side tool or similar tool mounted in a slowly advancing tool post shaves a thin sheet or ribbon from the end of the rod of powder. In 70 this manner, a maneuver powder suitable for use in the three-inch field gun and other mobile artillery guns and howitzers of greater and less calibers than three-inch, has been produced when the rod of powder 75 makes from 500 to 800 revolutions while the tool is advancing one inch. I do not limit myself to 500 to 800 revolutions per inch advance of the tool, as a greater or less number of revolutions will answer. The 80 same result may be obtained with the cutting tool or tools revolving and the powder advancing, or with the tool or tools revolving and advancing and the powder stationary, or with any other combination of 85 motions such that the relative motions of tool and powder are as above described.

I do not limit myself to the ordinary side tool or tools, as the powder may be produced among other ways, by mounting a 90 tool or tools in a holder of the type sometimes called "pencil sharpener." As previously indicated, the "pencil sharpener" may revolve and advance, or revolve only, or advance only, or be without motion, the 95 motion or lack of motion of the rod or piece of powder conforming thereto.

In the appended drawings, which form a part of this specification, Figure 1 is a perspective view of a suggestive device for carrying out the method of cutting with side tool; Fig. 2 is a side view illustrating a powder cutting tool of the pencil sharpener type; Fig. 3 is an end view of the form of tool shown in Fig. 2; Fig. 4 suggests another form of cutter in which successive blades traverse the entire face of the powder rod; Fig. 5 is a view in a direction at right angles to that of Fig. 4, showing a method of bringing a succession of shaving knives across the face of the powder rod, and Figs. 6 and 7 are an edge view and a face view, respectively, of still another form of cutter.

According to Fig. 1, the powder block 1 is rotated in position to have its end shaved 115 by the radially positioned tool 2 held in the post 3.

According to Figs. 2 and 3, knives 4 mounted upon a conical shell 5 in positions tangential to the inner wall of the shell, are adapted to cut shavings from the conical end of the powder stick 1, when the cutter is rotated through its shank 6 or held through said shank while the powder stick 120 is rotated.

According to Fig. 4, blades 7 to be held in any suitable manner in a mounting (not shown), between which and the powder stick 1 bodily movement takes place, are adapted 125 to cut shavings from the powder stick by 130

sweeping its entire transverse section at once.

According to Fig. 5, cutters 7<sup>a</sup> upon a rotary mounting 8, are adapted to shave the entire section of the powder stick by the passage of each cutter across its surface.

According to Figs. 6 and 7, face cutters 9, mounted in a rotary head 10, are adapted to shave chips from the end of the powder stick 1 with the same effect as described in connection with Figs. 4 and 5.

While not essential to my process, it is desirable that a spray or stream of water flow upon the tool or powder or both, while the powder is being cut to avoid the danger of fire from heating of the tool or piece of powder being cut.

It may or may not be necessary to dry the maneuver powder after it is cut, depending upon the composition of the rod or piece of explosive used in making the maneuver powder, or upon whether or not the powder is wet with water while being cut.

If a stick or cord of the same composition as what is known as straight nitrocellulose powder, is cut "green" or with a considerable amount of the solvents remaining in it, the maneuver powder will usually have to be dried before it will give the most satisfactory results in firing. If the stick or cord has already been dried so as greatly to reduce the moisture and volatile content, and the maneuver powder has not been wet in cutting, there may be no necessity for further drying.

Powders composed of mixtures of nitrocellulose and nitroglycerin when cut into maneuver powder usually require no further drying or but little drying, unless they have been wet while being cut. When drying is necessary, it may be accomplished in any of the usual ways. One satisfactory method is to place the powder in rooms or chambers, in which the temperature is raised to from 40° centigrade to 70° centigrade. I do not

limit myself to those temperatures as the powder may be dried satisfactorily at other temperatures. It may also be dried satisfactorily in other ways such as by desiccation, or by vacuum using various temperatures, or even by exposing to ordinary atmospheric temperature.

I claim:

1. A maneuver powder which, when fired with low confining resistance, will simulate in report and appearance, the discharge of a normal service charge; said powder consisting of sheets or disks cut from rods, sticks or other pieces of explosive of suitable composition, which strips, sheets or disks are relatively very thin as compared with their other dimensions, such as length and breadth, or diameter.

2. A maneuver powder which, when fired with low confining resistance, will simulate in report and appearance, the discharge of a normal service charge; said powder consisting of sheets or disks cut from rods, sticks or other pieces of explosive of suitable composition, which strips, sheets or disks are relatively very thin as compared with their other dimensions, such as length and breadth, or diameter; said strips, sheets, or disks being of a form developing a comparatively large bulk and occupying a space sufficient to constitute a safeguard against using, through error or accident, a dangerous large charge.

3. The herein described maneuver powder composed of shavings or chips of relatively thin dimension and of form developing a large bulk in comparison with its density, and having the qualities of developing, when lightly confined, a loud report with minimum visible products of combustion.

The foregoing specification signed at Dover, New Jersey, this 14th day of February, 1916.

JESSE C. NICHOLLS.

Copies of this patent may be obtained for five cents each, by addressing the "Commissioner of Patents, Washington, D. C."